

June 23, 1953

G. H. JONKER ET AL

2,643,192

ELECTRICAL INSULATOR

Filed June 11, 1949



|   | X  | Y  | Z  |
|---|----|----|----|
| a | 18 | -  | 82 |
| b | 16 | 19 | 65 |
| c | -  | 67 | 33 |
| d | 18 | 27 | 55 |
| e | 27 | 12 | 61 |
| f | 27 | -  | 73 |

MOL. %

GERARD HEINRICH JONKER AND  
PIETER BENEDICTUS ARIE SCHILPEROORD

BY

*Fred M. Vogel*

AGENT

INVENTORS

1/4 CaO

SrO

PbO

La<sub>2</sub>O<sub>3</sub>

## UNITED STATES PATENT OFFICE

2,643,192

## ELECTRICAL INSULATOR

Gerard Heinrich Jonker and Pieter Benedictus  
 Arie Schilperoord, Eindhoven, Netherlands,  
 assignors to Hartford National Bank and Trust  
 Company, Hartford, Conn., as trustee

Application June 11, 1949, Serial No. 98,546  
 In the Netherlands June 25, 1948

2 Claims. (Cl. 106—39)

## 1

*Improvements in or relating to electrical insulators*

This invention relates to electrical insulators. Ceramic products obtained by reaction of barium oxide with titanium dioxide are known. According to the molecular ratio of the said oxides in the initial mixture, it is possible to produce various barium titanates and mixtures thereof with titanium dioxide which exhibit divergent dielectric properties.

Of the compounds that may come into existence in the system  $\text{BaO}-\text{TiO}_2$ , barium metatitanate,  $\text{BaO} \cdot \text{TiO}_2$ , is particularly known on account of its extremely high dielectric constant ( $\epsilon$  greater than 1000). However, the tangent of the loss angle,  $\tan \delta$ , and the temperature coefficient of dielectric constant of barium metatitanate are too high for many uses.

Furthermore, it is known that barium tetratitanate,  $\text{BaO} \cdot 4\text{TiO}_2$ , may be produced. Barium tetratitanate has a much lower dielectric constant than barium metatitanate ( $\epsilon$  about 40) but has a lower  $\tan \delta$  and a temperature coefficient of dielectric constant of about  $+100 \cdot 10^{-6}$  per  $^{\circ}\text{C}$ .

It has now been found that in the system  $\text{BaO}-\text{TiO}_2$  a third compound barium trititanate,  $\text{BaO} \cdot 3\text{TiO}_2$ , may be formed, of which the dielectric constant and the  $\tan \delta$  approximately correspond with those of barium tetratitanate but of which the temperature coefficient is about  $-100 \cdot 10^{-6}$  per  $^{\circ}\text{C}$ .

An inconvenience in manufacturing ceramic insulators from mixtures consisting of  $\text{BaO}$  and  $\text{TiO}_2$  is that during sintering such mixtures do not readily react into a stable final state.

It has been found that the ternary system  $\text{ZnO}-\text{BaO}-\text{TiO}_2$  includes compositions which permit of obtaining valuable dielectrics by sintering or melting and which with regard to their working up differ from mixtures of  $\text{BaO}$  and  $\text{TiO}_2$  in that the desired stable final state is readily reached even at a comparatively low temperature and that a better sintering is obtained.

The invention will now be described with reference to the accompanying drawing in which:

Fig. 1 shows a ternary diagram defining regions in which preferred compositions of the invention will be found;

Fig. 2 shows a ternary diagram similar to Fig. 1 defining the entire region in which the compositions of the invention are found.

## 2

According to the invention, the said advantages are obtained in the first place with compositions forming products built up from mixed crystals located in the regions indicated in the accompanying ternary diagram (Fig. 1) by A and B, and also from mixtures of the said mixed crystals. The limits of the said mixed-crystal regions are dependent to a small extent on the temperature treatment chosen in the preparation. These mixed crystals may be regarded as barium tetratitanate and barium trititanate respectively in which a portion of the  $\text{Ti}^{IV}$ -ions is substituted by a substantially equivalent amount of  $\text{Zn}^{II}$ -ions.

Furthermore the said advantages are obtained with compositions forming products consisting of mixtures of zinc orthotitanate with these mixed crystals. In the phase diagram (Fig. 1) of the system  $\text{BaO}-\text{ZnO}-\text{TiO}_2$  included within lines I and II connecting the mixed-crystal regions A and B to the point corresponding to the composition of zinc orthotitanate are the compositions referred to previously. The region of compositions according to the invention does not include those which are built up from only two components.

The products obtained by sintering or melting and built up from mixed crystals located in the regions A and B, as well as those from the mixtures of the said mixed crystals have a  $\tan \delta$  lower than about  $5 \cdot 10^{-4}$  and a dielectric constant comprised between about 30 and 40, the temperature coefficient of dielectric constant frequently having decreased to values comprised between  $+50 \cdot 10^{-6}$  and  $-50 \cdot 10^{-6}$  per  $^{\circ}\text{C}$ .

By addition of zinc orthotitanate, which has a dielectric constant of about 20 and a temperature coefficient of dielectric constant of about  $+150 \cdot 10^{-6}$  per  $^{\circ}\text{C}$ ., the values of these properties may be modified. It is evident that this is attended with an increase of  $\tan \delta$  to the value thereof for zinc orthotitanate, viz. about  $20 \cdot 10^{-4}$ . With a product containing a high percentage of zinc orthotitanate and having the composition 6.5  $\text{BaO}-48.5 \text{ZnO}-45 \text{TiO}_2$  (point 14 in the diagram) the  $\tan \delta$  has, however, only decreased to about  $8 \cdot 10^{-4}$ .

In order to illustrate the invention, the table following hereinafter shows a number of products of different compositions the dielectric properties and the sintering temperatures used with these

compositions. The table also includes data for barium tetratitanate, barium trititanate and zinc orthotitanate.

At the most approximately half of the ZnO may furthermore be substituted by MgO. If a larger portion is substituted, a considerable in-

| No. | sintering temperature, °C. | composition in mol percent |      |                  | dielectric properties |                                                      |                       | final product                                      |
|-----|----------------------------|----------------------------|------|------------------|-----------------------|------------------------------------------------------|-----------------------|----------------------------------------------------|
|     |                            | BaO                        | ZnO  | TiO <sub>2</sub> | ε                     | $\frac{1}{\epsilon} \frac{d\epsilon}{dt} \cdot 10^6$ | tgδ · 10 <sup>4</sup> |                                                    |
| 1   | 1,320                      | 20                         | 0    | 80               | 43                    | +100                                                 | ca. -10               | BaO <sub>4</sub> TiO <sub>2</sub>                  |
| 2   | 1,320                      | 20                         | 5    | 75               | 38                    | -17                                                  | 0.5                   | mixed crystal A.                                   |
| 3   | 1,320                      | 18.5                       | 12.5 | 60               | 31                    | -                                                    | 1.5                   | mixed crystal A+TiO <sub>2</sub>                   |
| 4   | 1,320                      | 25                         | 0    | 75               | 42                    | -108                                                 | 3.5                   | BaO <sub>3</sub> TiO <sub>2</sub>                  |
| 5   | 1,300                      | 25                         | 5    | 70               | 35                    | -50                                                  | 1.4                   | mixed crystal B.                                   |
| 6   | 1,280                      | 23.5                       | 11.5 | 65               | 31                    | -                                                    | 4.3                   | Do.                                                |
| 7   | 1,320                      | 22.5                       | 2.5  | 75               | 41                    | -                                                    | 1.5                   | mixed crystal A+B                                  |
| 8   | 1,320                      | 20                         | 10   | 70               | 35                    | +22                                                  | 5.6                   | Do.                                                |
| 9   | 1,280                      | 21                         | 14   | 65               | 32                    | -                                                    | 1.5                   | Do.                                                |
| 10  | 1,250                      | 18                         | 20   | 62               | 34                    | +18                                                  | 1.6                   | mixed crystal A+B+Zn <sub>2</sub> TiO <sub>4</sub> |
| 11  | 1,250                      | 18                         | 22   | 60               | 30                    | -                                                    | 1.7                   | Do.                                                |
| 12  | 1,250                      | 13                         | 32   | 55               | 30                    | +45                                                  | 2.2                   | Do.                                                |
| 13  | 1,250                      | 10                         | 40   | 50               | 25                    | +90                                                  | 5.1                   | Do.                                                |
| 14  | 1,250                      | 6.5                        | 48.5 | 45               | 24                    | +100                                                 | 8                     | Do.                                                |
| 15  | 1,320                      | 4                          | 56   | 40               | 23                    | +165                                                 | 21                    | Do.                                                |
| 16  | 1,400                      | 0                          | 66.7 | 33.3             | 21                    | +160                                                 | 16                    | Zn <sub>2</sub> TiO <sub>4</sub>                   |

The  $\tan \delta$  increases very rapidly directly outside the region bounded by the lines I and II of the diagram (Fig. 1) and the mixed-crystal regions A and B. This seems to be connected with the production of free titanium dioxide or barium metatitanate in the final product. However, an excess of some mol. percent of  $\text{TiO}_2$  or  $\text{BaO}$  in the initial mixture need not necessarily have unduly detrimental consequences. With an increase of the content of  $\text{TiO}_2$  by less than about 2 mol. per cent or of  $\text{BaO}$  by less than about 4 mol per cent in the initial mixture,  $\tan \delta$  still remains below  $25 \cdot 10^{-4}$ . The region of compositions entering into consideration according to the invention extends, therefore, to the lines III and IV of the diagram and includes products containing a small amount of free  $\text{TiO}_2$  or  $\text{BaO} \cdot \text{TiO}_2$ , as illustrated in the following table:

crease in  $\tan \delta$  results, as is illustrated in the following table:

| composition in mol. percent |     |     |                  | dielectric properties |                                                      |                              |
|-----------------------------|-----|-----|------------------|-----------------------|------------------------------------------------------|------------------------------|
| BaO                         | ZnO | MgO | TiO <sub>2</sub> | $\epsilon$            | $\frac{1}{\epsilon} \frac{d\epsilon}{dt} \cdot 10^5$ | $\text{tg}\delta \cdot 10^4$ |
| 20                          | 20  | 0   | 60               | 31                    | +25                                                  | 1.1                          |
| 20                          | 15  | 5   | 60               | 28.5                  | +38                                                  | 1.3                          |
| 20                          | 10  | 10  | 60               | 23                    | +58                                                  | 1.9                          |
| 20                          | 5   | 15  | 60               | 28.5                  | +200                                                 | 141                          |
| 00                          | 0   | 20  | 60               | 26.5                  | +320                                                 | 195                          |

Furthermore,  $ZnO$  may be substituted by  $BeO$  in such manner that the content of  $BeO$  is about 35 mol % at the most. It is to be noted that if  $ZnO$  is substituted completely by  $BeO$ , a great excess of  $TiO_2$  is permissible without a

| No. | sintering<br>temp.,<br>°C. | composition in mol.<br>percent |     |                  | dielectr.<br>properties |                     | final product                     |
|-----|----------------------------|--------------------------------|-----|------------------|-------------------------|---------------------|-----------------------------------|
|     |                            | BaO                            | ZnO | TiO <sub>2</sub> | ε                       | tgδ·10 <sup>4</sup> |                                   |
| 17  | 1,300                      | 17                             | 15  | 68               | 30                      | 25                  | mixed crystal+TiO <sub>2</sub>    |
| 18  | 1,300                      | 27                             | 3   | 70               | 43.5                    | 18                  | mixed crystal+Ba.TiO <sub>3</sub> |
| 19  | 1,280                      | 27                             | 8   | 65               | 45                      | 24                  | mixed crystal+Ba.TiO <sub>3</sub> |
| 20  | 1,250                      | 25                             | 15  | 60               | 36                      | 24                  | mixed crystal+Ba.TiO <sub>3</sub> |

In the region of compositions according to the invention the constituents may be partly substituted isomorphously by other oxides without appreciable influence on the dielectric properties, if this substitution takes place in such manner that the product obtained remains built up substantially from zinc-containing mixed crystals of barium tetra titanate and/or barium trititanate or mixtures of zinc orthotitanate with these mixed crystals.

ZnO may be substituted by CdO in such manner that the content thereof is 5 mol. % at the most, as is illustrated in the following table:

high  $\tan \delta$  resulting. The dielectric constant is then greater, but the temperature coefficient, which is negative, is also greater. Examples of BeO substitution are illustrated in the following table:

| Composition in mol. percent |       |     |                  | dielectric properties |                                                      |                              |
|-----------------------------|-------|-----|------------------|-----------------------|------------------------------------------------------|------------------------------|
| BaO                         | ZnO   | BeO | TiO <sub>2</sub> | $\epsilon$            | $\frac{1}{\epsilon} \frac{d\epsilon}{dt} \cdot 10^6$ | $\text{tg}\delta \cdot 10^4$ |
| 20                          | 4     | 4   | 72               | 34                    | -18                                                  | 6.3                          |
| 20                          | ----- | 5   | 75               | 34                    | -40                                                  | 0.4                          |
| 22                          | ----- | 8   | 70               | 33                    | -----                                                | 3.9                          |
| 18                          | ----- | 20  | 62               | 30                    | -----                                                | 1.0                          |
| 10                          | ----- | 20  | 70               | 42                    | -230                                                 | 1.8                          |
| 10                          | ----- | 10  | 80               | 39                    | -260                                                 | 3.8                          |

Substitution of the BaO by oxides such as CaO, SrO, PbO and La<sub>2</sub>O<sub>3</sub>, which may produce metatitanates but which cannot produce trititanates and tetratitanates, is possible to a limited extent. The type of the mixed crystals and mixtures would undergo undue variation if large

quantities were to be substituted. Notably, free metatitanate would be produced so that  $\tan \delta$  would attain unduly high values. With substitution of a quarter at the most of the BaO by one or more of the said oxides, the  $\tan \delta$  still remains below  $25.10^{-4}$ , as is illustrated in the following table:

| composition in mol. percent |     |     |     |                                    |     |                  | dielectric properties |                                                      |                          |
|-----------------------------|-----|-----|-----|------------------------------------|-----|------------------|-----------------------|------------------------------------------------------|--------------------------|
| BaO                         | SrO | CaO | PbO | $\frac{1}{2}\text{La}_2\text{O}_3$ | ZnO | TiO <sub>2</sub> | $\epsilon$            | $\frac{1}{\epsilon} \frac{d\epsilon}{dt} \cdot 10^6$ | $\tan \delta \cdot 10^4$ |
| 21                          | 3   | --- | --- | ---                                | 6   | 70               | 34                    | ---                                                  | 0.5                      |
| 18                          | 6   | --- | --- | ---                                | 6   | 70               | 38                    | ---                                                  | 6.8                      |
| 14                          | 5   | --- | --- | ---                                | 19  | 62               | 38.5                  | -300                                                 | 2.1                      |
| 15                          | 8   | --- | --- | ---                                | 2   | 75               | 37                    | -390                                                 | 4.4                      |
| 14                          | 5   | --- | --- | ---                                | 19  | 62               | 38                    | -195                                                 | 2.0                      |
| 18                          | --- | --- | 4   | ---                                | 10  | 68               | 30                    | ---                                                  | 3                        |
| 19                          | --- | --- | --- | 2                                  | 8   | 71               | 31                    | ---                                                  | 4.9                      |

Finally, it is possible that about a quarter at the most of the TiO<sub>2</sub> is substituted by compounds such as ZrO<sub>2</sub>, SnO<sub>2</sub> and SiO<sub>2</sub>. Examples of ZrO<sub>2</sub>, SnO<sub>2</sub> and SiO<sub>2</sub> substitution are illustrated in the following table:

| Composition in mol. percent |     |                  |                  |                  |                  | dielectric properties |                          |
|-----------------------------|-----|------------------|------------------|------------------|------------------|-----------------------|--------------------------|
| BaO                         | ZnO | TiO <sub>2</sub> | ZrO <sub>2</sub> | SnO <sub>2</sub> | SiO <sub>2</sub> | $\epsilon$            | $\tan \delta \cdot 10^4$ |
| 22                          | 8   | 55               | 15               | ---              | ---              | 25                    | 7.0                      |
| 22                          | 8   | 60               | ---              | 10               | ---              | 36                    | 17                       |
| 22                          | 8   | 55               | ---              | ---              | 15               | 24                    | 5.6                      |

It is to be understood that one of the constitutive oxides may be substituted isomorphously by a plurality of oxides simultaneously. An example thereof is the composition 15 BaO—4 SrO—10 ZrO<sub>2</sub>—3 MgO—3 BeO—64 TiO<sub>2</sub>. The sintered product thus obtained has  $\epsilon=32$  and  $\tan \delta=7.10^{-4}$ .

Fig. 2 shows a ternary diagram similar to Fig. 1 illustrating schematically the principal constituents of the compositions according to the invention and the partially replacing oxides for each constituent.

The invention which is based on the foregoing relates to an electrical insulator consisting of a mass, obtained by sintering or melting, substantially built up from zinc-containing mixed crystals of barium tetra titanate and/or barium trititanate or mixtures of zinc orthotitanate with these mixed crystals, it being possible that one or more of the constitutive oxides are substituted isomorphously by other oxides to such extent that the mass still substantially consists of mixed crystals or mixtures of the said type and has a  $\tan \delta$  smaller than  $25.10^{-4}$ , preferably smaller than  $10.10^{-4}$ .

The insulators according to the invention are suitable more particularly for use in the manufacture of condensers.

The invention further relates to a method of preparing an insulating substance on the basis of the above-described mixed crystals or mixtures by mixing of the initial substances, for example in a ball mill, and subsequent heating.

Besides the constitutive oxides themselves also compounds of these oxides, such as titanates, and compounds which change to the oxides concerned on application of heat may be used as initial materials.

The heating process is performed in a neutral or oxidising atmosphere in such manner that the conversions into the desired mixed crystals

and mixtures are obtained to such extent that unduly large amounts of free TiO<sub>2</sub> or metatitanate are not contained in the final product and as a consequence thereof the value  $\tan \delta$  is below  $25.10^{-4}$ . The heating process is preferably continued until a stable final state is obtained at the temperature used. Dependent

on the composition, the initial mixtures will sinter upon heating at temperatures comprised between about 1250 and 1350° C. and melt at temperatures below 1450° C.

It is, in addition, possible to utilise in known manner mineralisers such as CaF<sub>2</sub>, sintering agents such as bentonite or steatite, and binders such as nitrocellulose.

It is of importance that, possibly due to the strong tendency to formation of mixed crystals of the compositions according to the invention, impurities may readily be absorbed by the crystal lattice and do not, in general, tend to give rise to the formation of a separate phase in the final product. Consequently, the purity of the initial materials need not satisfy extremely stringent requirements. For example, with compositions from which products having a  $\tan \delta$  smaller than  $10.10^{-4}$  are produced, such as 25 BaO—5 ZnO—70 TiO<sub>2</sub>, the  $\tan \delta$  is increased only to approximately  $22.10^{-4}$  due to the presence of oxides such as MnO<sub>2</sub>, Cr<sub>2</sub>O<sub>3</sub>, NiO to an amount of approximately 3% by weight.

The insulating substance thus obtained may be used, after having been pulverised, for the manufacture of so-called drawn condensers which, as is known per se, may be obtained in that a plurality of coaxial conductors between which insulating material is provided, is subjected to a treatment for the purpose of decreasing the diameter, such as a swaging or drawing treatment.

What we claim is:

1. A ceramic dielectric consisting essentially of a ternary composition defined wholly within the region of the phase diagram of the ternary system X—Y—Z shown in Fig. 2 of the accompanying drawing bounded by angular points having the composition 18X—82Z, 16X—19Y—65Z, 67Y—33Z, 18X—27Y—55Z, 27X—12Y—61Z and 27X—73Z calculated in mol. per cent, where X includes BaO and one of the oxides selected from the group consisting of CaO, SrO, PbO and La<sub>2</sub>O<sub>3</sub> in an amount not exceeding one quarter of the BaO, Y includes ZnO and not more than 5 mol. per cent of CdO, not more than 35 mol. per cent of BeO and not more than 50 mol. per cent MgO, and Z includes TiO<sub>2</sub> and one of the oxides selected from the group consisting of ZrO<sub>2</sub>, SnO<sub>2</sub> and SiO<sub>2</sub> in an amount not exceeding one quarter of the TiO<sub>2</sub>.

2. A ceramic dielectric consisting essentially of a ternary composition defined wholly within the region of the phase diagram of the ternary system X—Y—Z shown in Fig. 2 of the accom-

7

panying diagram bounded by angular points having the composition 18X—82Z, 16X—19Y—65Z, 67Y—33Z, 18X—27Y—55Z, 27X—12Y—61Z and 27X—73Z calculated in mol. per cent, where X consists of BaO, Y consists of ZnO, and Z consists of TiO<sub>2</sub>.

Number  
2,220,765  
2,277,734  
2,369,327

5

| Name          | Date          |
|---------------|---------------|
| Hirose et al. | Nov. 5, 1940  |
| Wainer et al. | Mar. 31, 1942 |
| Wainer        | Feb. 13, 1945 |

8

## FOREIGN PATENTS

| Country       | Date |
|---------------|------|
| Great Britain | 1946 |

GERARD HEINRICH JONKER.  
PIETER BENEDICTUS ARIE SCHILPEROORD. Number  
574,577

References Cited in the file of this patent 10

## UNITED STATES PATENTS

| Number    | Name  | Date          |
|-----------|-------|---------------|
| 2,071,452 | Block | Feb. 23, 1937 |